

July 28, 1953

P. D. WILLIAMS

2,647,067

ELECTRON Emitter FOR ELECTRON TUBES

Filed Sept. 10, 1949



Fig. 1

INVENTOR.  
PAUL D. WILLIAMS  
BY *Harold E. Eng*

ATTORNEY

## UNITED STATES PATENT OFFICE

2,647,067

## ELECTRON Emitter FOR ELECTRON TUBES

Paul D. Williams, Palo Alto, Calif., assignor to  
 Eitel-McCullough, Inc., San Bruno, Calif., a  
 corporation of California

Application September 10, 1949, Serial No. 114,958

1 Claim. (Cl. 117—33.28)

1

My invention relates to an electron emitter or cathode for electron tubes, such as transmitting type vacuum tubes.

It is among the objects of my invention to provide an emitter having the desired electron emission properties of a thoriated type tungsten emitter, but which is made from ordinary tungsten metal suitably treated rather than from the prepared thoriated tungsten heretofore employed.

Another object is to provide an emitter which may be fabricated in any suitable shape, including surface type cathodes as well as wire type filaments.

The invention possesses other objects and features of advantage, some of which, with the foregoing, will be set forth in the following description of my invention. It is to be understood that I do not limit myself to this disclosure of species of my invention as I may adopt variant embodiments thereof within the scope of the claim.

Referring to the drawing:

Figure 1 is an elevational view of an electron tube embodying a filamentary type cathode of my invention, portions of the internal parts being broken away to show the structure more clearly; and

Figure 2 is a detailed view showing the emitter filament.

In terms of broad inclusion, my improved electron emitter comprises a tungsten core, and a coating comprising an intimate mixture of tungsten and thorium oxide sintered on the core. The preferred method of making the emitter comprises reducing thorium tungstate to a mixture of tungsten and thorium oxide, coating the core with the mixture, and sintering the coating onto the core. Either wire or sheet-like core metal may be used, depending upon whether the emitter is to be of the filamentary or the surface type cathode.

In greater detail and referring to the drawing, a triode type of filamentary cathode tube is chosen for purposes of illustration, it being understood that my improved emitter may be incorporated in tubes other than triodes. It is also understood that the emitter may be of the unipotential surface type rather than the filamentary type shown. The tube illustrated comprises an evacuated glass envelope 2 with a stem 3 carrying an exhaust tubulation 4 and provided with a base 6 having terminal prongs 7. Stem 3 is formed separately from the envelope 2 and is finally sealed to the envelope after the electrodes have been mounted, as is conventional practice. The envelope encloses a filamentary cathode 8

hereinafter described in detail, a tubular metal anode 9 and a cage-like wire grid. Anode 9 has a cap 12 supported by a bracket 13 on lead 14 sealed to the upper end of the glass envelope.

5 A pair of leads 17 sealed to stem 3 support the cathode, which leads are connected to a pair of base prongs 7 by conductors 18. The grid 11 has a base ring 21 supported by brackets 22 on a pair of rods 23 sealed to the stem 3, one of these rods 10 being connected by a conductor 24 to the base prong. Figure 2 shows the filamentary cathode or emitter more clearly, the helical filament being connected at its ends to the leads 17. At the time the filament is mounted on the leads 17, the 15 glass stem 3 has not been sealed to the envelope 2, so that the filament stem assembly may be handled separately from the remaining portions of the tube during processing of the filament.

My improved emitter of Figure 2 comprises a 20 tungsten core wire coated with an intimate mixture of finely divided tungsten metal and thorium oxide sintered on the core. The tungsten used for the core of the filament 8 may be an ordinary commercial grade of substantially pure tungsten 25 wire and is suitably formed into helical shape and secured to the leads 17. The preferred procedure then comprises reducing thorium tungstate to a mixture of metallic tungsten and thorium oxide, coating the tungsten core with such mixture, and sintering the coating onto the core. The preparation of the coating mixture from thorium tungstate is an important step in the procedure, because it provides the desired 30 intimate mixture of very finely divided tungsten metal and thorium oxide.

35 Reduction of the thorium tungstate is preferably accomplished by placing a quantity of thorium tungstate powder in a suitable container and heating it in a hydrogen atmosphere to a temperature of about 1000° C. This results in the partial reduction of the thorium tungstate compound to metallic tungsten and thorium oxide. As hereinbefore mentioned, the advantage of forming the mixture by this reduction 40 process is that the resulting particles of tungsten metal and thorium oxide are in a finely divided state and are uniformly distributed to provide an intimate mixture.

45 The resulting product, which is a fine black powder, is then mixed with a liquid binder, such as amyl acetate, to a consistency suitable for application, as by spraying, on the core of filament 8. A spray coat about .0005 inch thick on the wire core is satisfactory.

50 55 The coated filament is then heated in vacuum

to about 2300° to 2500° C. brightness temperature to sinter the coating. This sintering may conveniently be accomplished by passing current through the filament while the filament stem is in an evacuated bell jar. After sintering, the filament is carburized and otherwise treated in the usual manner of handling ordinary thoriated tungsten filaments.

For example, the filament is preferably carburized by heating it in a suitable hydrocarbon atmosphere to a temperature of say 2100° C. to 2400° C. brightness. The purpose of carburizing is to introduce carbon into the filament, by the formation of tungsten carbide, which carbon is then available for reducing the thorium oxide to metallic thorium during operation of the filament.

After carburization, the grid 11 is mounted in place and the completed filament stem is sealed in the envelope. Thereafter, the tube is evacuated in the usual manner.

As hereinbefore mentioned, my improved emitter may be fabricated as a unipotential or surface type cathode. In this case a sheet of tungsten is used as the core instead of tungsten wire. A 25 convenient shape is a cylinder of sheet tungsten having its outer surface coated as above described

for the wire filament. This cylindrical cathode may be heated indirectly by a suitable heater within the cylinder in the usual manner of heating indirectly heated cathodes.

5 I claim:

An electron emitter element for use in an electron tube comprising a tungsten core having sintered thereon a coating consisting essentially of an intimate mixture of metallic tungsten and 10 thorium oxide, said coating mixture being formed by the reduction of thorium tungstate in a hydrogen atmosphere at a temperature of about 1000° C.

15 PAUL D. WILLIAMS.

References Cited in the file of this patent

UNITED STATES PATENTS

| Number    | Name     | Date           |
|-----------|----------|----------------|
| 1,608,317 | Hyde     | Nov. 23, 1926  |
| 1,896,614 | Gehrts   | Feb. 7, 1933   |
| 2,269,081 | Felsner  | Jan. 6, 1942   |
| 2,339,392 | Garner   | Jan. 18, 1944  |
| 2,438,732 | Williams | Mar. 30, 1948  |
| 2,447,038 | Spencer  | Aug. 17, 1948  |
| 2,450,007 | Litton   | Sept. 28, 1948 |